

## UNITED STATES PATENT OFFICE

FRITZ STRAUB, OF BASEL, SWITZERLAND, AND HERMANN SCHNEIDER, OF RIEHEN NEAR BASEL, SWITZERLAND, ASSIGNORS TO SOCIETY OF CHEMICAL INDUSTRY IN BASEL, OF BASEL, SWITZERLAND

## PROCESS FOR DYEING ANIMAL FIBERS FAST TINTS

No Drawing. Application filed September 15, 1930, Serial No. 482,155, and in Switzerland September 26, 1929.

The present invention relates to a process for dyeing animal fibers fast tints. It comprises the new dyeing process, as well as the material dyed according to the new process.

- 5 It is known that the chromium compounds or other metal compounds of azo-dyestuffs containing groups capable of being metallized have acquired considerable importance in the wool dyeing industry in that they permit the production of well equalized tints of 10 remarkable fastness on wool or other animal fiber by merely dyeing in a sulfuric acid bath. However, dyeing in a sulfuric acid bath does not attain the desired object in the case of 15 the chromium compounds of azo-dyestuffs of the general formula

20



wherein R stands for a naphthol. These dyestuffs are precipitated in the sulfuric acid bath before they are absorbed by the fiber so that there are obtained weak dyeings which are not fast. If it is attempted to dye the material with these dyestuffs in an organic acid bath, the dyestuff can be completely absorbed on the fiber but the correct depth of dyeing or the valuable properties of fastness or both are not attained.

The present invention is based on the surprising observation that it is possible to dye animal fibers with the dyestuffs of the above mentioned general formula fast tints by first dyeing the fiber in a weakly acid bath and then converting the dyestuff absorbed by the fiber into new complexes by developing it in the same dye-bath by heating or boiling, which bath is made stronger acid by the addition of an acid.

At the initial dyeing operation from a weakly acid bath, in which the dyestuff is absorbed by the fiber completely or partially, the addition of organic acids, as for example formic acid, acetic acid, oxalic acid, is expedient, but there may also be used inorganic acids if these latter are added slowly and

in small quantities to the dyeing bath.

In the second stage of the new dyeing process, i. e. in developing, a new dyestuff complex is formed. It must be carried out in a stronger acid bath. For this purpose additions of 55 inorganic acids, such as sulfuric acid, hydrochloric acid, are particularly suitable, but the use of organic acids, if these are added in larger quantities, also leads to good results.

The essential moment for the success of the 60 present dyeing process resides in the fact that in the developing bath the dissociation of the added acid must be farther advanced than in the initial dyeing bath, i. e. the pH of the developing bath must be smaller than the pH of 65 the dyeing bath. It is known that in the case of non-metalliferous dyestuffs capable of dyeing in presence of organic acids the absorption of the dyestuffs can be completed by the addition of a mineral acid at the end of 70 the dyeing process. The process in accordance with the present invention, however, differs from the aforesaid procedure in that it comprises the further development of dyestuffs which are present on the fibre or, respectively, their conversion into other complexes. 75

The following examples illustrate the invention, the parts being by weight:

## Example 1

The dye-bath is prepared from 2000 parts of water, 5-6 parts of formic acid, which may if desired be added in portions during dyeing, and 3-4 parts of the chromium compound of the dyestuff of the formula



obtainable as described in Example 1 of the copending specification Serial No. 482,364 95 filed September 16, 1930. 100 parts of wool are entered into the bath at 90°C. Dyeing is continued for a quarter of an hour and the temperature is then raised to boiling in the course of a further 1/2 hour. This tem- 100

perature is maintained for some time until the dyestuff is absorbed, whereupon 6-7 parts of concentrated sulfuric acid are added and the bath is boiled until the dyestuff is completely developed, this operation requiring about  $\frac{3}{4}$  to 1 hour. The wool is thereby dyed a deep black tint of very good fastness properties.

It is also possible to conduct the dyeing 10 using from the start sulfuric acid alone, if care be taken that before the dyestuff is absorbed the pH value of the dye-bath is not substantially less than that of the dye-bath containing the formic acid; this may be obtained by adding mineral acid to the bath very slowly and gradually or by adding a formate to the bath at the commencement.

*Example 2*

20 The printing color is prepared by dissolving 20 parts of the chromium compound obtainable as described in Example 1 of the co-pending specification Serial No. 482,364 filed September 16, 1930 and 60 parts of neutral 25 starch tragacanth thickening in 380 parts of water. The material is printed with this printing color in the usual manner. After drying it is steamed for 1 hour in a Mather-Platt apparatus at an over-pressure of  $\frac{1}{4}$  30 atmosphere, then it is rinsed with water and finished in the usual manner. There are thus obtained on wool or silk black prints of very good fastness properties.

What we claim is:—

35 1. Process for dyeing animal fibers fast tints, consisting in first dyeing the fiber in a weakly acid bath with the chromium compounds of azo-dyestuffs of the general formula



wherein R stands for naphthol, and then converting the dyestuff absorbed by the fiber into new complexes by developing it in the same bath which is made stronger acid by the addition of an acid.

50 2. Process for dyeing animal fibers fast tints, consisting in first dyeing the fiber in a weakly acid bath with the chromium compound of the azo-dyestuff of the formula



and then converting the dyestuff absorbed by the fiber into new complexes by developing it in the same bath which is made stronger acid by the addition of an acid.

3. Process for dyeing animal fibers fast tints, consisting in first dyeing the fiber in an organic acid bath with the chromium compound of the azo-dyestuff of the formula



and then converting the dyestuff absorbed by the fiber into new complexes by developing it in a bath which is made stronger acid by the addition of an acid.

4. Process for dyeing animal fibers fast tints, consisting in first dyeing the fiber in an organic acid bath with the chromium compound of the azo-dyestuff of the formula



and then converting the dyestuff absorbed by the fiber into new complexes by developing it in the same bath which is made stronger acid by the addition of an inorganic acid.

5. Process for dyeing animal fibers fast tints, consisting in first dyeing the fiber in a bath containing formic acid with the chromium compounds of the azo-dyestuff of the formula



and then converting the dyestuff absorbed by the fiber into new complexes by developing it in the same bath which is made stronger acid by the addition of an inorganic acid.

6. Process for dyeing animal fibers fast tints, consisting in first dyeing the fiber in a bath containing formic acid with the chromium compound of the azo-dyestuff of the formula



and then converting the dyestuff absorbed by the fiber into new complexes by developing it in the same bath which is made stronger acid by the addition of sulfuric acid.

In order whereof we have hereunto signed our names this 6th day of September 1930.

FRITZ STRAUB.  
HERMANN SCHNEIDER.